

## UNITED STATES PATENT OFFICE

GARLAND H. B. DAVIS, OF BATON ROUGE, LOUISIANA, ASSIGNOR TO STANDARD OIL DEVELOPMENT COMPANY, A CORPORATION OF DELAWARE

## HYDROCARBON OIL AND PROCESS FOR MANUFACTURING THE SAME

No Drawing.

Application filed May 3, 1930. Serial No. 449,693.

The present invention relates to improved methods for the production of high grade lubricating oils and more specifically comprises such products as new composition of matter and improved methods for their manufacture.

In the production of high grade lubricating oils it is well known that low solidification or pour points are highly desirable, particularly with motor oils or oils which are adapted for machinery operating at low temperatures, for example; ice machine oil and the like. There are methods at the present time for reducing the pour point of lubricating oils and these ordinarily consist of freezing the oil and separating the solidified paraffinic material by filtration or by centrifugal action, but these methods are extremely expensive.

Another highly desirable property for lubricating oils is a relatively small change in the viscosity between temperatures of say 210° F. and 100° F. In other words, it is desirable for the oil to approach the Pennsylvania type of lubricating oil in which the viscosity-temperature curve is relatively flat, rather than to approach the Texas or Colombian type of oil in which viscosity changes very rapidly with temperature change.

Hereafter the phrase "high quality" will be used to designate oils having the desirable relatively flat temperature-viscosity curve and "low quality" for oils at the other extreme, such as Texas coastal oils, irrespective of other properties usually necessary to a superior lubricant. As used here "quality" is equivalent to viscosity index as defined by Dean and Davis in their article in Chemical and Metallurgical Engineering, vol. 36, page 618.

I have found that the presence of paraffin or other waxy hydrocarbon materials tends to improve the quality of an oil and that the same oil after paraffin has been removed will be more or less inferior in respect to its viscosity-temperature characteristics. It is, therefore, highly desirable to keep solidifiable paraffinic materials in the oil from the point of view of desirable temperature-viscosity characteristics, but at the same time

the presence of such materials is undesirable with respect to solidification or pour points, as will be understood.

I have discovered methods by which paraffin containing oils, such as those obtained from Pennsylvania or equivalent crudes or Mid-Continent crudes of the intermediate type, or even from low grade crudes, which have been improved in quality by the addition of petrolatum or paraffin wax, may be greatly improved with respect to their pour or solidification points without detriment to quality. This is likewise of particular importance with oils produced by hydrogenation of heavy carbonaceous materials, since pour points of such products are frequently high. This may be accomplished at a low cost and without expensive refrigeration methods. I have found that certain materials added to these oils have the power of depressing or otherwise reducing the pour point of the oil as determined by the standard test method given in "Report on petroleum products and lubricants and methods for tests relating to petroleum products" by the committee D-2 of the American Association of Testing Materials, and published in 1928. The method appears on page 83 and the following pages of this report.

In the use of my method I first chlorinate a paraffinic material such as paraffin wax, petrolatum or other aliphatic hydrocarbons, either pure or in a mixed state, by means of passing chlorine therethru while at a temperature between about 140 and 300° F. for a prolonged period after which it is found that the paraffin contains 10 to 12% chlorine, or more. Other materials as indicated above may be used in place of paraffin wax and such materials are chosen which contain relatively long aliphatic hydrocarbon chains. Aromatic hydrocarbon material such as naphthalene or anthracene or the like is then mixed with, say an equal weight of aluminum chloride and the chlorinated oil is slowly added while maintaining a low condensation temperature of about 140 to 160° F. The proportion of the chlorinated product to the aromatic material may vary considerably say from .10 to .50 parts of the latter to 1.0 of

55

60

65

70

75

80

85

90

95

100

the former. The mixture is kept in constant agitation and it is highly desirable to have present some solvent, say a light hydrocarbon predominately saturated, such as kerosene or the like. The reaction may be carried out at room temperature and under such conditions it takes a somewhat longer time, say about 24 hours. It is desirable at the end of the time to raise the temperature slowly to about 200° F. to complete the reaction and throughout copious volumes of hydrochloric acid vapors are allowed to escape from the treating vessel. Instead of a solid aromatic hydrocarbon other materials rich in cyclic hydrocarbons may be used, for example; benzol or toluol, although in this case it is particularly desirable to carefully prevent undue rise in temperature. Aromatic gas oils such as those occurring in the California crudes and particularly tube and tank cycle stock such as is produced from cracking crudes or gas oils are also satisfactory, particularly California cycle oil and the like.

The oil mixture is then allowed to stand for a considerable time to allow sludge constituents to settle and the oil is withdrawn and cooled. It is preferable at this time to remove a part or all of the unreacted paraffin and this may be done by cold pressing or other similar methods, although distillation under high vacuum is preferred. The unreacted wax is removed as a vapor, leaving the synthetic oil as a residue. The synthetic oil may then be blended with the wax-bearing oil in any desirable proportion, say less than 10% or 5%, or even 1%, if it is merely desired to reduce the pour point of the paraffin containing stock, or it may be added in larger quantities, say from 10 or 20 to 30 or even to 50% where it is desired to improve the quality of the product i. e. with respect to its viscosity-temperature characteristics. It will be found that the blended oil has a greatly reduced pour point as determined by the standard test method referred to above, even when less than 1% of the synthetic oil is added and if larger amounts of the synthetic oil are added to low quality oils with relatively steep viscosity-temperature curves it will be found that the blend has a viscosity-temperature curve, the slope of which is considerably reduced and brought nearer to the ideal type of lubricating oil represented by Pennsylvania oil. In addition the oil is given an attractive green color and bloom characteristic of the highest grade oils.

As an example of the operation of my process and the production of my improved lubricating oils the following is given. A hard paraffin wax having a melting point of 122 to 125° F. is chlorinated by the direct addition of chlorine in the presence of a trace of iodine and at a temperature of about 200° F. The chlorine is blown through the oil for

about 24 hours and after this time it is found that the product contains about 12% chlorine, which correspond to a predominant quantity of the mono-chlor derivative although there is usually some unchlorinated hydrocarbon. To 90 parts of this chloro-paraffin 10 parts of naphthalene and 10 parts of aluminum chloride are then added with a sufficient quantity of kerosene to completely dissolve the organic materials. The reaction is carried on at room temperature and is found to be substantially complete in about 24 hours and at this time the temperature is raised gradually to about 200° F. The aluminous sludge is then allowed to settle and the liquid oil is withdrawn and distilled to remove the kerosene and the unreacted paraffin as distillates. The heavy oil remaining has the following inspection:

|                   |                   |    |
|-------------------|-------------------|----|
| Gravity           | 23.4° A. P. I.    | 85 |
| Vis. at 100° F.   | 8500 sec. Saybolt |    |
| Vis. at 210° F.   | 312 sec. Saybolt  |    |
| Pour              | 65° F.            |    |
| Flash             | 535° F.           |    |
| Conradson carbon  | 4.6%              |    |
| Residual chlorine | .2%               |    |

A vacuum distilled Mid-Continent oil has the following inspection:

|                 |                   |    |
|-----------------|-------------------|----|
| Gravity         | 24.7° A. P. I.    | 90 |
| Vis. at 100° F. | 981 sec. Saybolt  |    |
| Vis. at 210° F. | 79.3 sec. Saybolt |    |
| Flash           | 515° F.           |    |
| Pour            | 35° F.            |    |
| Carbon          | .409%             |    |

A blend is then made up of 90% of the vacuum distilled Mid-Continent lubricating oil and 10% of the synthetic oil and the inspection of the blend is as follows:

|                 |                   |     |
|-----------------|-------------------|-----|
| Gravity         | 24.5° A. P. I.    | 100 |
| Vis. at 100° F. | 1077 sec. Saybolt |     |
| Vis. at 210° F. | 86 sec. Saybolt   |     |
| Flash           | 515° F.           |     |
| Pour            | below 10° F.      |     |
| Carbon          | .935%             |     |

It will be observed that the pour point of the oil has been greatly reduced and the quality of the oil has been improved.

As a second example a distillate from Pennsylvania crude has the following characteristics:

|                 |                   |     |
|-----------------|-------------------|-----|
| Gravity         | 28.9° A. P. I.    | 110 |
| Vis. at 100° F. | 433 sec. Saybolt  |     |
| Vis. at 210° F. | 60.5 sec. Saybolt |     |
| Flash           | 445° F.           |     |
| Pour            | above 30° F.      |     |
| Carbon          | .50%              |     |

and is blended with 1% of a synthetic oil similar to that used in the first example and the blend shows the following inspection:

|                 |                   |     |
|-----------------|-------------------|-----|
| Gravity         | 28.8° A. P. I.    | 120 |
| Vis. at 100° F. | 450 sec. Saybolt  |     |
| Vis. at 210° F. | 61.5 sec. Saybolt |     |
| Pour            | below 5° F.       |     |
| Flash           | 450° F.           |     |
| Carbon          | .570%             |     |

This blended oil is found to be stable over a long period of time, showing no separation or deterioration.

As a third example, a Colombian lubricating distillate after treatment with 5 pounds of 66° Bé. sulphuric acid and having

been filtered with 5 pounds of clay per barrel of oil has the following inspection:

|   |                 |                   |  |
|---|-----------------|-------------------|--|
| 5 | Gravity         | 23.8° A. P. I.    |  |
|   | Vis. at 100° F. | 479 sec. Saybolt  |  |
|   | Vis. at 210° F. | 56.5 sec. Saybolt |  |
|   | Flash           | 410° F.           |  |
|   | Pour            | 0° F.             |  |
|   | Carbon          | 152%              |  |

This oil is blended with a synthetic oil similar to that used in Example 1, except that it had a viscosity of 239 sec. Saybolt at 10 210° F. and a pour of 70° F. and with petrolatum of 31° A. P. I. gravity and having a viscosity of 43 sec. Saybolt at 210° F. The addition of the petrolatum causes the pour 15 point of the Colombian oil and petrolatum mixture to be considerably higher than the pour point of the Colombian oil alone, but when the three components are blended in proportions of 85% of the Colombian lube distillate, 5% synthetic oil and 10% petrolatum the blended product has the following inspection:

|    |                 |                   |  |
|----|-----------------|-------------------|--|
| 25 | Gravity         | 24.5° A. P. I.    |  |
|    | Vis. at 100° F. | 457 sec. Saybolt  |  |
|    | Vis. at 210° F. | 57.5 sec. Saybolt |  |
|    | Pour            | below -10° F.     |  |
|    | Carbon          | 34.7%             |  |
|    | Flash           | 410° F.           |  |

It will be observed in this case that the pour point is held at a low figure in spite of the fact that 10% petrolatum was added to the 30 oil and that the slope of the viscosity temperature curve was greatly reduced.

As a fourth example 3 parts of a hydrogenated Colombian lubricating oil is blended with 1 part of the synthetic oil described in 35 Example 1. Inspections of the Colombian oil and the blend is given below:

|    |                               |          |               |
|----|-------------------------------|----------|---------------|
| 40 | Hydro-generated Colombian oil | Blend    |               |
|    | Gravity A. P. I.              | 27.5°    | 27.2°         |
|    | Visc. at 100° F. (Saybolt)    | 246 sec. | 442 sec.      |
|    | Visc. at 210° F. (Saybolt)    | 47 sec.  | 60.5 sec.     |
| 45 | Pour                          | 0° F.    | Below -10° F. |
|    | Flash                         | 410° F.  | 440° F.       |

A particularly desirable feature of my invention comprises the use of narrow cut lubricating oils to be blended with the synthetic oil. These oils may be produced by 50 fractionation or by ordinary vacuum distillation. Due to the narrow boiling range of the particular cut it is endowed with a relatively high flash in comparison with its viscosity, and if it is obtained from sweet crudes 55 it is usually rich in paraffin having a high pour point often above 50° F. It is desirable to reduce the pour by the ordinary commercial methods, such as filtration to about 50 or preferably to 30° F. and to blend thereof 60 with from 1 to 5% of the synthetic oil described above. This blend is particularly desirable in that it is found to have an abnormally high flash point for its viscosity at 210° F. and a pour below 10° F. or even 65 below zero.

As an example of this type of oil the following tests are given:

|  |                               |             |                    |
|--|-------------------------------|-------------|--------------------|
|  | Hydro-generated Colombian oil | 1% blend    | 70                 |
|  | Gravity A. P. I.              | 27.4        | 27.3               |
|  | Vis. at 100° F. (Saybolt)     | 495         | 500                |
|  | Vis. at 210° F. (Saybolt)     | 60          | 61                 |
|  | Pour                          | 30          | Below minus-20° F. |
|  | Flash                         | 480         | 480                |
|  | Boiling range 10 mm. of Hg.   | 500-600° F. | 75                 |

This invention is not to be limited by any theory of the mechanism of the reactions, nor to any specific example which may have 80 been given for the purpose of illustration, but only by the following claims in which I wish to claim all novelty inherent in my invention.

I claim:

1. An improved lubricating oil comprising 85 a blend of a viscous hydrocarbon fraction containing a solid waxy constituent in proportion sufficient to give a relatively high pour point and a synthetic hydrocarbon oil 90 formed by the condensation of a waxy hydrocarbon material with an aromatic hydrocarbon.

2. A lubricating oil according to claim 1 in which the viscous hydrocarbon is a hydro- 95 genated product.

3. An improved lubricating oil comprising 100 a blend of a heavy viscous hydrocarbon fraction containing a waxy constituent in proportion sufficient to give a relatively high pour point with a synthetic hydrocarbon oil obtained by condensation of a waxy hydrocarbon with a solid aromatic hydrocarbon, the synthetic oil being in pour reducing proportions only.

4. An improved lubricating oil with a pour 105 point below 10° F. comprising a blend of a viscous hydrocarbon having a pour point above 30° F. with an effective quantity of a synthetic hydrocarbon obtained by condensation of paraffin with an aromatic hydrocarbon.

5. An improved lubricating oil with a pour 115 point below 0° F. comprising a blend of a viscous hydrocarbon having a pour point above 10° F. with an effective quantity of a synthetic hydrocarbon obtained by condensation of paraffin with an aromatic hydrocarbon.

6. An improved lubricating oil of relatively 120 low pour point comprising a blend of a petroleum fraction of relatively higher pour point with a minor proportion of a synthetic oil formed by the condensation of paraffin wax with an aromatic hydrocarbon.

7. An improved lubricating oil of relatively 125 low pour point comprising a blend of a petroleum fraction of relatively higher pour point with a synthetic oil formed by the condensation of paraffin wax and a solid

- aromatic hydrocarbon, the synthetic oil being in pour reducing proportion, but below 10% and effective substantially only for pour reduction.
5. 8. An improved lubricating oil of relatively low pour point comprising a blend of a petroleum fraction of relatively higher pour point with a synthetic oil formed by the condensation of paraffin wax and a solid aromatic hydrocarbon, the synthetic oil being in pour reducing proportion, but below 5% and effective substantially only for pour reduction.
10. 9. An improved lubricating oil of relatively low pour point comprising a blend of a petroleum fraction of relatively higher pour point with a synthetic oil formed by the condensation of paraffin wax and a solid aromatic hydrocarbon, the synthetic oil being in pour reducing proportion, but below 1% and effective substantially only for pour reduction.
15. 10. An improved lubricating oil of relatively low pour point comprising a blend of a petroleum fraction of relatively higher pour point with a synthetic hydrocarbon oil in proportion effective for pour reduction only, the synthetic oil being a low temperature aluminum chloride condensation product of halogenated paraffins and an aromatic hydrocarbon.
20. 11. An improved lubricating oil of relatively low pour point comprising a blend of a petroleum fraction of relatively higher pour point with a synthetic hydrocarbon oil in proportion effective for pour reduction only, the synthetic oil being a low temperature aluminum chloride condensation product of chlorinated paraffin wax and naphthalene.
25. 12. An improved lubricating oil of relatively low pour point comprising a blend of a petroleum fraction of relatively higher pour point with a synthetic hydrocarbon oil in proportion effective for pour reduction only, the synthetic oil being a low temperature, aluminum chloride condensation product of mono-chlor paraffin wax and naphthalene.
30. 13. An improved lubricating oil of low pour point comprising a hydrocarbon oil of higher pour point with a synthetic hydrocarbon in an effective proportion of the order of 1%, the synthetic oil being a low temperature, aluminum chloride condensation product of mono-chlor paraffin wax and naphthalene.
35. 14. An improved lubricating oil of relatively low pour point comprising a viscous petroleum hydrocarbon of relatively higher pour point with a synthetic hydrocarbon in an effective proportion of the order of 1%, the synthetic oil being a low temperature, aluminum chloride condensation product of mono-chlor paraffin wax and naphthalene.